

Jan. 14, 1941.

L. SIMONS

**2,228,916**

## METHOD OF MAKING AN ALLOY

Filed May 10, 1937

2 Sheets-Sheet 1



Fig: 4



Fig: 3

INVENTOR.

*Seon Simons*

Mock & Blum

BY

ATTORNEYS.

Jan. 14, 1941.

L. SIMONS

2,228,916

METHOD OF MAKING AN ALLOY

Filed May 10, 1937

2 Sheets-Sheet 2

Fig: 5



Fig: 6



Fig: 7



INVENTOR.  
*Leon Simons*  
BY  
*Block & Blum*

ATTORNEYS.

## UNITED STATES PATENT OFFICE

2,228,916

## METHOD OF MAKING AN ALLOY

Leon Simons, New York, N. Y.

Application May 10, 1937, Serial No. 141,618

5 Claims. (CL. 75—137)

My invention relates to a new and improved method of making bodies of hard and refractory material. The invention also relates to an improved hard and refractory material.

One of the objects of my invention is to make bodies of material which include tungsten carbide, and other compounds or elements which have high melting points.

Another object of my invention is to make an improved material of the type which includes tungsten carbide or other ingredient which has a high melting point, and which also includes an additional metal having a lower melting point than said tungsten carbide. This additional metal may be cobalt or nickel or other metal, or alloy having a melting point which is lower than the ingredient which has the high melting point. The ingredient which has the high melting point preferably comprises at least 50% by weight of the improved material, although the ingredient which has the lower melting point, such as cobalt or nickel, may be present in any desired proportion.

Another object of my invention is to provide a material having a higher proportion of nickel or cobalt or the like, than has hitherto been practical.

Another object of my invention is to provide an improved method of making an alloy which includes tungsten or tantalum or other metal having a high melting point.

Another object of my invention is to provide an improved hard alloy which includes tungsten carbide or tantalum carbide or other carbides which have high melting points.

The finished product which is made according to my invention may consist of minute particles of tungsten carbide or other carbides, which have been melted while in contact with cobalt or nickel or other material having a lower melting point than the carbide, and which has been recrystallized from said melt. This application is in part a continuation of application Serial No. 35,039, filed in the United States Patent Office on August 7, 1935, now Patent No. 2,151,874, dated Mar. 28, 1939.

Alloys or cemented carbides of the type which I desire to improve, are described in Schrotter U. S. Reissue Patent No. 17,624 and in numerous other patents such as U. S. Patent No. 1,895,364, U. S. Patent No. 1,895,354, U. S. Patent No. 1,892,653, U. S. Patent No. 1,937,185, U. S. Patent No. 1,950,356, French Patent No. 573,624, and others.

The invention relates to the improvement of

alloys or cemented carbides of any of the said types, or containing any of the ingredients specified in said patents, and it also generally applies to the manufacture of any type of alloy.

Other objects of my invention will be set forth in the following description and drawings which illustrate a preferred embodiment thereof, it being understood that the above statement of the objects of my invention is intended generally to explain the same without limiting it in any manner.

Fig. 1 shows the first step in the improved method.

Fig. 2 diagrammatically shows apparatus which can be used for carrying out the second step of my method.

Fig. 3 is a detail sectional view, partially in elevation, showing how the particles of tungsten carbide or the like can be enclosed in a metal shell which is closed at one end and which is open at the other end, in using the apparatus which is shown in Fig. 2.

Fig. 4 shows another method of impinging the particles of tungsten carbide or the like against a mass of nickel or cobalt or other auxiliary metal.

Fig. 5 is a microphotograph, made under a magnification of 1500, showing material which has been fused and allowed to cool, according to the method specified herein, without the use of pressure.

Fig. 6 is a microphotograph, at the magnification above stated, showing the improved material made according to the best embodiment of the invention, and with the use of heat and pressure.

Fig. 7 is a microphotograph made at the magnification above stated and showing the starting material which is used for making the improved material.

Heretofore, in making alloys of the old type which consisted of minute particles of tungsten carbide, said particles were cemented together with cobalt or nickel, according to the old process, which was a sintering process. In such old sintering process, the proportion of nickel or cobalt did not exceed about 18% to 20% by weight of the tungsten carbide. The sintering process was not practical, with less than about 5% by weight of the nickel or cobalt, because the use of a lower percentage resulted in a product which had voids.

According to my invention, the tungsten carbide or equivalent material is preferably reduced to a particle size which is much finer than the particle size which has heretofore been employed,

when a sintering mixture was made according to the prior art.

The usual practice has been to make such particles sufficiently fine to pass through a No. 320 screen. A screen which is designated as No. 320 has 320 holes per linear inch and these holes are substantially equally spaced. Hence the particle size, according to the old method was about .0015 inch, (fifteen ten-thousandths of an inch).

10 According to my invention I reduce the tungsten carbide or the like much more finely so that the particles are as fine as 0.0002 inch (two ten-thousandths of an inch). While I do not wish to be limited to such very fine particle size, this 15 will serve as a practical working figure. The particles may be even finer.

I then coat these fine particles of tungsten carbide or the like, intimately and sufficiently with the cobalt or nickel or additional metal or material. By using very fine particles, having large surface areas in proportion to their volumes, I can coat the fine particles with sufficient additional metal. For this purpose and in order to lower cost of manufacture and to secure a 25 sufficient and even coating, I prefer to project the particles of tungsten carbide with sufficient velocity against a mass or body of nickel or cobalt or the like. For this purpose, and as shown in Fig. 1, the particles of tungsten carbide can be projected by means of air pressure or other fluid pressure, through a tube 1, and the particles are projected at high velocity against a body 2, which is made of nickel or cobalt or the like. Said body 2 may be held horizontally 30 or vertically or in any position.

The air pressure which is utilized for projecting the particles of tungsten carbide may be derived from a source of compressed air whose pressure is as high as one hundred pounds per 40 square inch or even higher.

I do not wish to be limited to any particular velocity of the projected tungsten carbide particles, and said velocity may be as high as is desired.

45 As shown in Fig. 1, the particles of tungsten carbide may glance off the stationary mass of nickel or cobalt and such particles are coated sufficiently with nickel or cobalt or the like, which is removed by impact or abrasion from

50 the solid mass of nickel or cobalt. Some of the particles of tungsten carbide may be imbedded in the mass of nickel or cobalt or the like and such particles can be readily removed from the mass of nickel or cobalt or the like, by means of 55 a scraping action, which will finely divide the nickel or cobalt or the like.

Likewise I can utilize apparatus of the general type which is exemplified in U. S. Patent No. 2,032,827 dated March 3, 1936, whereby the 60 particles of tungsten carbide are projected at high velocity against an annular member made of nickel or cobalt or the like.

In passing through said apparatus, the particles of tungsten carbide repeatedly strike the 65 annular body of nickel or cobalt, and the particles of tungsten carbide are repeatedly deflected from the annular member made of nickel or cobalt.

This operation continued in one or more 70 stages until the particles of tungsten carbide have taken up the required percentage or percentages of additional metal or material. If a tungsten carbide alloy is to be made, the percentage of nickel or cobalt which is taken up 75 may be as low as five per cent or even two per

cent, and as high as twenty-five percent or even higher.

I generally include within the invention alloys of the type above mentioned, containing tungsten carbide or other refractory material or refractory carbide, and having more than eighteen percent of an additional metal having a lower melting point than the tungsten carbide or the like.

10 I include generally any step in the manufacture of any alloy whereby particles of metal or alloy, of any size, are caused to impact with coating-metal material. For example, projected particles of tungsten carbide and of nickel can be caused to collide with each other, while said 15 particles are moving at high velocity. This is to be distinguished from the operation of a ball mill or the like in which the particles of tungsten carbide and nickel are merely rubbed against each other but without any impact or 20 abrasive action.

As shown in Fig. 4, the particles P can be projected at a high velocity from the tube T, against the wall of a recess n of the large stationary mass N, which may be made of nickel or cobalt 25 or the like. The projected particles of tungsten carbide or the like are moved in the path shown, so as to rub off sufficient nickel or cobalt or the like, which clings to said fine particles.

After the fine particles of tungsten carbide 30 or the like have been sufficiently coated with the coating metal, I can use any suitable process to form a coherent mass from said particles.

However, I prefer to use the process and apparatus illustrated in Fig. 2, although the improved 35 process can be used with any type of apparatus.

Fig. 2 shows, a base 1 made of steel or other metal. The upper surface of the base 1 is provided with a covering member A which is made of asbestos or of other material which is extremely refractory and which has high heat-insulating properties. Member A is preferably rigid and it may be made of the material known to the trade as "rock asbestos".

The upper surface member A is provided with a recess, in which a filling 3 is located. Said filling 3 is also made of refractory and heat-insulating material. Said filling 3 may consist of a mixture of lamp black and of silica.

45 The filling 3 is in the form of a dense and coherent block which has been made by subjecting a mixture of lamp black and silica to suitable pressure. The filling 3 can withstand pressure which is as high as one thousand pounds per square inch or even higher. The filling 3 is utilized because it is a better heat insulator than the block A and it is desired to utilize material which has maximum heat-insulating properties and which is extremely refractory, as the working temperature may be as high as 2600° C. 60 The block A closes the lower end of casing 2 which is made of suitable refractory material. Casing 2 can be made of quartz or of fused-alumina material of the type which is known as "alundum".

Above the top surface of the block A, casing 2 can be filled with material 9 in finely divided powder form. Said material 9 can have the same composition as the filling material 3 so that filling material 9 has maximum heat-insulating properties.

While the material 9 is subjected to pressure during the operation of the device, said material 9 remains substantially in loose and powdered form.

The block A' is identical with the block A and it has a dense coherent filling 3' which is identical with the filling 3 of the block A.

A graphite mould 4 is provided with a bottom planar surface which rests on top of the block 3. The block 3 projects outwardly beyond the bottom of the mould 4, through a distance which is sufficiently so as to provide for efficient heat insulation. This distance may be an eighth of 10 an inch or as much more as is desired.

Suitable means are provided for preventing the mould 4 from shifting laterally relative to the block 3. For example, the adjacent surfaces of the block 3 and of the mould 4 can be provided with interfitting projections and recesses. The interior of the graphite mould 4 is filled with the coated tungsten carbide material or the like.

Plunger 8 has a cylindrical bottom portion which fits slidably and very closely in the cylindrical bore of the recessed upper portion 6 of the mould 4. The plunger 8 is also made of graphite and suitable means are provided for preventing any lateral shift between plunger 8 and block 3'. Said means can consist of suitable interfitting recesses and projections. The block 3' is identical with the block 3 and it is located in the recess of a movable member A', which is identical with the member A.

Block A' is subjected to pressure by any suitable means such as removable weights 10.

In compressing the material 7, this being the coated tungsten carbide or the like, I can use pressures as high as four thousand pounds per square inch. The material 7 is located in the field of the hollow coil G which is supplied with a suitable high frequency current. This high frequency current may have a frequency as high as seventy thousand cycles per second and the voltage which is induced or produced at the ends 40 of the coil G may be as high as 1000 volts.

While I do not wish to be limited to any specific temperatures, as these may depend upon the material which is being treated, the material 7 is generally heated to a temperature between 45 2500° C. and 2600° C., if the material which is being treated is tungsten carbide, which has been coated with about fifteen per cent of nickel. However, the temperature may be lower and it may even be higher, depending upon the type 50 of material which is being treated in the apparatus which is disclosed in Fig. 2.

The coil G may be cooled by forcing water or other cooling medium through the same, and for this purpose the coil G has an inlet end 11 55 and an outlet end 12. Said coil G also has its ends provided with electric couplings 14' and 15' to which the electrical leads 14 and 15 are connected. Said leads 14 and 15 are connected to a high frequency converter or any other suitable source of high frequency current.

After the apparatus has been assembled, some pressure, less than the maximum working pressure, is applied to the plunger 8. This initial pressure may be about one-half of the maximum 65 working pressure, which may be as high as 4000 pounds per square inch.

As soon as the initial pressure has been applied to plunger 8, current is supplied to the coil G. The graphite mould 4 is preferably, but 70 not necessarily, of the type which is sufficiently porous or absorbent so as to cause the driving out of the air or other gases which are intermixed with the material 7, and some of the nickel or cobalt may also enter the wall of the recessed 75 portion of the mould 4. Indeed the working

temperature may be so high as to cause a portion of the tungsten carbide material or the like to enter the material of the mould 4. For this purpose the mould 4 may be made of graphite of the relatively porous type of graphite used for 5 making the brushes of dynamos or the like. Graphite of this relatively porous type is also used for making ultra fine filters. The wall of the recess of the mould 4 may have a thickness of from one-quarter of an inch to three-quarters 10 of an inch, depending upon the diameter of the recess.

While Fig. 2 is diagrammatic, it is substantially according to scale.

The high frequency current heats the material 7 by means of induction. In order to permit the proper heating of the material 7, it may contain and it preferably does contain a small percentage of iron which may be as high as two per cent. This iron or other paramagnetic 20 material may be incorporated into the particles before they are coated with nickel or cobalt or the like. The iron or other auxiliary paramagnetic material may be omitted.

It is believed that the heating effect is due in part to conduction, in part to the alternating magnetic polarity of the particles, and in part by eddy currents, and also by hysteresis. It is also believed to be due in part to electrostatic 25 induction.

The particles of the material 7 therefore fuse so that the volume of the material 7 can be diminished by the pressure. This additional pressure is applied quite rapidly so that a slug of material is formed from the material 7 and the 30 height of said slug is about twenty-five per cent less than the original height of the material.

The entire process should not take from more than five minutes to eight minutes and preferably less time, as for example three minutes or 40 even less.

After the plunger 8 has descended to its lowest position, the current supply of the coil G is switched off. After the current supply has been discontinued, the material can be maintained 45 under the maximum pressure for a suitable period, such as fifteen minutes, until the material 7 has solidified.

The close fit of plunger 8 in the recess of the mould, causes the material 7 to be maintained in 50 a space which is substantially air-tight, during the heat and pressure treatment. Likewise the material is treated quite rapidly so that any oxidation of the tungsten carbide or other oxidizable material is substantially prevented, without using an inert or reducing atmosphere, although such atmosphere could be used.

While the material is being heated and subjected to pressure, the coil G can be continuously cooled so as to maintain said coil at a temperature of about 50° F.

After the current supply has been discontinued, the cooling effect of the coil G can be continued. The coil G is preferably spaced from the member 65 2, which is made of material which is a good insulator against both heat and electricity.

The above directions are mainly for making a slug which can be used for making a die for drawing wire.

The final material consists predominantly of 70 tungsten carbide crystals (containing iron or the like), if the starting material was coated tungsten carbide. These tungsten carbide crystals are regular in shape, indicating recrystallization from solid solution.



The maximum pressure utilized was 2000 pounds per square inch.

The first step was to apply a pressure of 500 pounds per square inch and then to supply the heating current to the coil G. The pressure was then increased to 2000 pounds per square inch. The original particle size of the tungsten carbide powder which was used as a starting material was 0.0002 inch (two ten-thousandths of an inch). This original starting material had 10% by weight of cobalt.

Upon analyzing the final material which resulted from the use of this starting material, it was found that about 12% of the weight of the original starting material had been lost. When the original starting material had 10% by weight of cobalt, analysis showed that the final material illustrated in Fig. 6 had about 2.62% by weight of cobalt. Since the total loss of the material was 12% by weight of the original mass, the material lost 7.38% of the cobalt and 2.62% by weight of the tungsten carbide.

The material shown in Fig. 6 has a structure which consists of small to medium-sized crystals of tungsten carbide, showing recrystallization of the tungsten carbide.

The material shown in Fig. 6 also has a matrix which consists of a solid solution of tungsten-carbide-cobalt and the proportion of this matrix is small. The material illustrated in Fig. 6 differs mainly from the material illustrated in Fig. 5 by the complete absence of the voids which are shown in Fig. 5.

Likewise in Fig. 5 nearly all the crystals are of medium size, whereas the material illustrated in Fig. 6 has crystals of tungsten carbide which vary in size from the small size to the medium size.

A comparison between Fig. 5 and Fig. 6 and Fig. 7, shows the difference in the crystals of tungsten carbide, due to the recrystallization thereof by the method above specified. In making the material illustrated in Fig. 6, the time of operation was from seven minutes to 8 minutes.

It will be noted that according to the improved method, the refractory material, such as tungsten carbide, is initially physically associated with a metal having a lower melting point than said refractory material and that some of this low-melting metal is eliminated from the refractory material, during the heating operation above specified.

It is believed that the addition of a relatively large percentage of cobalt to the initial material, by the method above specified, makes it possible to lower the melting point of the mixture so that the operating temperature need not exceed 2200° C. to 2300° C.

I can produce a final alloy of the type shown in Fig. 6, and having any desired percentage of nickel or cobalt or the like, by incorporating a sufficiently large percentage of nickel or cobalt or the like into the starting material.

Likewise the elimination of nickel or cobalt or the like from the refractory material, can be controlled by regulating the working temperature, or the time of operation, or the porosity of the graphite mould or the like.

There are certain types of graphite which are extremely dense so that the elimination of nickel or cobalt or the like is much less than if the graphite is relatively porous.

Whenever I refer to an alloy in the claims, it is to be understood that I intend to cover the

material illustrated in Fig. 5 or in Fig. 6, and which consists essentially of masses or crystals of the refractory material, held in a matrix which consists of a solid solution of the refractory material, and an auxiliary metal having a lower melting point than said refractory material.

I do not wish to be limited to any particular method of heating the coated refractory particles.

It will be noted that according to the preferred method the particles are subjected to heat and pressure without any substantial stirring action.

I have shown a preferred embodiment of my invention, but it is clear that numerous changes and omissions can be made without departing from its spirit.

The graphite plunger 8 may be very dense, so that little or no material enters it, or said plunger may have the same structure as the graphite mold. I claim:

1. In the art of making an alloy which includes a major proportion of a metallic carbide whose melting point exceeds 2000° C. and a minor proportion of a metal whose melting point is below 2000° C., in an enclosed mold having a movable ram which projects from a wall of said mold, those steps which consist in heating said metallic carbide and said metal in said mold while exerting pressure on the heated material by moving said ram, while compressing powdered material externally around said ram and said mold at said wall of the mold to hinder the entry of air between said ram and the adjacent wall portion of the mold, and then cooling the heated and pressed material in said mold.

2. In the art of making an alloy which includes a major proportion of a metallic carbide whose melting point exceeds 2000° C. and a minor proportion of a metal whose melting point is below 2000° C., in an enclosed mold having a movable ram which projects from a wall of said mold, those steps which consist in heating said metallic carbide and said metal in said mold while exerting pressure on the heated material by moving said ram, while compressing powdered material externally around said ram and said mold at said wall of the mold to hinder the entry of air between said ram and the adjacent wall portion of the mold, and then cooling the heated and pressed material in said mold, said metallic carbide being crystalline, the heating temperature being sufficiently high to recrystallize said metallic carbide during said cooling.

3. In the art of making an alloy which includes a major proportion of a metallic carbide whose melting point exceeds 2000° C. and a minor proportion of a metal whose melting point is below 2000° C., in an enclosed mold having a movable ram which projects from a wall of said mold, those steps which consist in heating said metallic carbide and said metal in said mold while exerting pressure on the heated material by moving said ram, while compressing powdered material externally around said ram and said mold at said wall of the mold to hinder the entry of air between said ram and the adjacent wall portion of the mold, and then cooling the heated and pressed material in said mold, said metallic carbide and said metal being heated by subjecting them to a varying electro-magnetic flux which induces a secondary voltage having a closed circuit within said carbide and said metal and the wall of the mold.

4. In the art of making an alloy which includes a major proportion of a metallic carbide whose melting point exceeds 2000° C. and a minor pro-

portion of a metal whose melting point is below 2000° C., in an enclosed mold having a movable ram which projects from a wall of said mold, those steps which consist in heating said metallic carbide and said metal in said mold while exerting pressure on the heated material by moving said ram, while compressing powdered material externally around said ram and said mold at said wall of the mold to hinder the entry of air between said ram and the adjacent wall portion of the mold, and then cooling the heated and pressed material in said mold, said metallic carbide being crystalline, the heating tempera-

ture being sufficiently high to recrystallize said metallic carbide during said cooling, said metallic carbide and said metal being heated by subjecting them to a varying electro-magnetic flux which induces a secondary voltage having a closed circuit within said carbide and said metal and the wall of the mold.

5. A method according to claim 1, in which the metal is in the form of a coating on the metallic carbide, and the metallic carbide is in the form of particles whose average diameter does not exceed 0.0002 inch.

LEON SIMONS.